

April 24, 1951

F. G. CIAPETTA

2,550,531

REFORMING PROCESS AND CATALYST THEREFOR

Filed Dec. 29, 1949

4 Sheets-Sheet 1

FIG. 1



FIG. 2



ATTEST

Cluwood J. Schaffer

INVENTOR.

FRANK G. CIAPETTA

BY

Robert E. Birch

ATTORNEY

April 24, 1951

F. G. CIAPETTA

2,550,531

REFORMING PROCESS AND CATALYST THEREFOR

Filed Dec. 29, 1949

4 Sheets-Sheet 2



ATTEST

Elwood J. Schaffer

INVENTOR.

FRANK G. CIAPETTA

BY Robert E. Bush

ATTORNEY

April 24, 1951

F. G. CIAPETTA

2,550,531

REFORMING PROCESS AND CATALYST THEREFOR

Filed Dec. 29, 1949

4 Sheets-Sheet 3



ATTEST

Clwood J. Schaffer

INVENTOR.

FRANK G. CIAPETTA  
BY Robert E. Bush

ATTORNEY

April 24, 1951

F. G. CIAPETTA

2,550,531

REFORMING PROCESS AND CATALYST THEREFOR

Filed Dec. 29, 1949

4 Sheets-Sheet 4

FIG. 6



ATTEST

Elwood J. Schaffer

INVENTOR.

FRANK G. CIAPETTA

BY Norbut E. Buch

ATTORNEY

## UNITED STATES PATENT OFFICE

2,550,531

REFORMING PROCESS AND CATALYST  
THEREFORFrank G. Ciapetta, Llanerch Hills, Pa., assignor  
to The Atlantic Refining Company, Philadelphia, Pa., a corporation of Pennsylvania

Application December 29, 1949, Serial No. 135,736

11 Claims. (Cl. 196—50)

1

This invention relates to a reforming process and to a reforming catalyst having particular surface area characteristics. More particularly it relates to a silica alumina catalyst, having a surface area from about 10 to about 65 square meters per gram, impregnated with platinum or palladium and to a process for reforming petroleum hydrocarbons with said catalyst to obtain high yields of products having high anti-knock properties.

The hydrocarbons to be treated in the invention comprise petroleum distillates, including naphthas, gasoline and kerosine, and particularly gasoline fractions. The gasoline fraction may be a full boiling range gasoline having an initial boiling point within the range of about 50° to about 90° F. and an end boiling point within the range of about 375° to about 425° F., or it may be a selected fraction thereof which usually will be a higher boiling fraction, commonly referred to as naphtha, and generally having an initial boiling point of from about 150° to about 250° F. and an end boiling point within the range of about 350° to about 425° F.

The petroleum hydrocarbons to be reformed are mixtures containing for the most part paraffinic hydrocarbons which are usually straight chain or slightly branched chain structures and cyclic compounds (so-called naphthenic hydrocarbons), especially cyclohexanes, as well as, in most cases, varying proportions of aromatic hydrocarbons. To obtain best results in reforming such hydrocarbons it is desirable to cause maximum isomerization of the paraffins to increase the amount of branched chain paraffins and isomerization of alkylcyclopentanes to cyclohexanes and dehydrogenation of the cyclohexanes to aromatics, selective cracking of the high molecular weight paraffins into lower molecular weight paraffins which are liquid at ordinary temperatures and dehydrocyclization of the paraffins to aromatics. At the same time it is desirable to keep at a minimum or to obtain substantially no demethanation of the paraffins during isomerization, hydrogenation of aromatics to naphthenic hydrocarbons and indiscriminate or uncontrolled cracking, particularly of the paraffins.

All the reactions during reforming are to a greater or lesser degree reversible depending on the various equilibria involved. The reversal of the dehydrogenation reaction of the cyclo compounds to aromatics takes place most readily and the reversal of the cracking reaction is most difficult particularly if carbon is formed during the cracking. The isomerization of the paraffins

5 in such hydrocarbon mixtures is one of the important factors in reforming them. During isomerization methyl and to a lesser extent ethyl groups are shifted from the straight chain to side chain positions and this should be done with a minimum of demethanation and/or carbon production. The carbon to carbon bonds instead of being broken are merely put under a strain in which condition, particularly in the presence of 10 the instant catalyst, they shift to the side chain position or positions to produce an isomer in which the carbon atoms are more centralized as compared to a straight chain compound. Such isomers have higher anti-knock characteristics 15 than their corresponding straight chain paraffins. Still another important series of reactions is the isomerization of alkyl cyclopentanes to cyclohexanes followed by the dehydrogenation of these cyclohexanes together with those originally 20 present in the mixture to aromatics. An additional means of forming aromatics is the dehydrocyclization of acyclic paraffins. These reactions result in an increase in the anti-knock characteristics of the reformed products since the 25 octane rating of aromatics is very high compared to that of the saturated cyclo compounds. Selective cracking of the long chain paraffins into low boiling fractions particularly when the charging stock contains components boiling above 30 about 400° F. is also important both because such lower boiling fractions by virtue of their lower molecular weights have higher octane numbers and because such lower boiling components may be further increased in anti-knock value by the 35 above described reactions.

The isomerization, however, should be accomplished with a minimum of demethanation and carbon deposition both because demethanation reduces yields and carbon deposition affects 40 catalytic activity further reducing yield. The presence of hydrogen during the reforming decreases the demethanation reaction and when a carbon to carbon bond is broken as when the higher molecular weight paraffins are cracked 45 or when a methyl or ethyl group is broken off the paraffin, the hydrogen saturates the carbon and in the case of the ethyl or methyl groups forms the corresponding gas and thereby prevents or greatly reduces the deposition of carbon. These 50 reactions are in reality hydrogenation reactions and take place simultaneously with the dehydrogenation that occurs with the dehydrocyclization of the paraffins and the aromatization of the saturated cyclo compounds.

55 It has been discovered that a silica-alumina

catalyst having a particular surface area and impregnated with platinum or palladium, displays a maximum isomer yield from open chain paraffins during the catalytic reforming of these compounds with such a catalyst. It has been discovered further that the maximum isomer yield obtainable with such catalysts having certain surface areas is extremely sensitive to temperature when the surface area of the component upon which the platinum or palladium is composited is greater than about 65 square meters per gram of component, that with surface areas smaller than this value the catalyst is substantially insensitive to temperature in so far as obtaining maximum isomer yield is concerned and that the change in sensitivity to temperature is so great at a surface area of about 65 square meters per gram of component as to be of critical importance in the reforming of hydrocarbons. These discoveries, together with the fact that increased temperature during reforming increases the aromatizations of saturated cyclohexanes and the dehydrocyclization of acyclic paraffins to aromatics permit the reforming of hydrocarbons to obtain reformed products which are high in yield and anti-knock value. By controlling the surface area of the catalyst high isomer yields at high temperatures can be accomplished during reforming regardless of pressure, since isomerization is independent of the pressure. This permits the use of high reaction temperatures which in turn favors maximum production of aromatic hydrocarbons. Moreover, since isomerization is independent of the pressure, higher hydrogen partial pressures at higher pressure may be used to reduce the amount of demethanation and carbon deposition, thus further contributing to the high yield of high octane products and increased life of the catalyst without regeneration. The applicant has also discovered that at surface areas of 10 square meters per gram of silica alumina component and below, the activity of the catalyst drops off rapidly and therefore surface areas from about 10 to about 65 square meters per gram of component should be used in practicing the invention.

Broadly the invention relates to a catalyst containing a cracking component having a surface area from about 10 to about 65 square meters per gram impregnated with platinum or palladium, said component comprising silica and alumina and to a process for treating petroleum distillates under reforming conditions with such catalyst.

In its narrower aspect, the invention relates to a catalyst containing a cracking component having a surface area from about 10 to about 65 square meters per gram comprising silica and alumina impregnated with platinum or palladium in amount from 0.01 to 2.5% by weight of the final catalyst and to a process for reforming a gasoline fraction with such catalyst at temperatures in the range 600 to 1000° F., at pressures in the range 100 to 1000 pounds per square inch, at an hourly liquid space velocity of from 0.1 to 10 in the presence of from 1 to 20 mols. of hydrogen per mol. of hydrocarbon. Larger or smaller amounts of platinum or palladium than in the range 0.01 to 2.5% by weight of the final catalyst may be used. Such larger or smaller amounts are not preferred, however, since amounts less than 0.01% result in too low an activity and in amounts larger than 2.5% result in excessive cracking.

The low surface area component upon which the platinum or palladium is deposited will have

some activity to catalyze the cracking reaction; however, this activity is low compared with the high surface area catalyst normally used in the cracking art. This is an important feature of the invention. This component may be derived either from naturally occurring or synthetically produced materials. Naturally occurring materials include various aluminum silicates, particularly when acid treated to increase the activity, such as Super Filrol, etc. The synthetic materials may be made in any suitable manner including separate, successive or co-precipitation of silica and alumina. The synthetic component, the area of which is preferably subsequently reduced, may be manufactured by commingling an acid, such as hydrochloric acid, sulfuric acid, etc., with commercial water glass under conditions to precipitate silica, washing with acidulated water or otherwise to remove sodium ions, commingling with an aluminum salt such as aluminum chloride, aluminum sulfate, aluminum nitrate, and either adding a basic precipitant, such as ammonium hydroxide, to precipitate alumina or forming the desired oxide or oxides by thermal decomposition of the salt as the case may permit. The cracking component may contain from 20-95 percent by weight of silica with the remainder alumina although amounts above and below this range may also be used. The component may be in the form of regular beads or granules of irregular size and shape. The granules may be ground and formed into pellets of uniform size and shape by pilling, extrusion or other suitable methods. Components prepared in this manner have surface areas of the order of magnitude of 400 square meters or more per gram.

It is preferable to adjust the surface area of the component at this point, i. e., before composing the platinum or palladium thereon, to the desired value in any suitable manner. This may be accomplished by steaming the component at temperatures of from 900 to 1400° F. at steam pressures from atmospheric to 100 pounds per square inch or higher for a sufficient time, usually for about 50 to 100 hours although longer or shorter periods may be used, to obtain the desired surface area or by heating the component at temperatures from 1600 to 1800° F. without the use of steam and for a sufficient time to obtain the desired surface area. The term surface area as used herein means the surface area of the component as determined by the adsorption of nitrogen according to the method of Brunauer, Emmett and Teller found in the Journal of the American Chemical Society, vol. 60, pages 309 et seq. (1938).

The platinum or palladium may be composited with the cracking component, prepared as above described, in any suitable manner. The preferred method is to admix with the cracking component an aqueous solution of chloro-platinic acid or a chloro-palladic acid of suitable concentrations in the desired amounts. The mixture is then dried and treated with hydrogen at elevated temperatures to reduce the chloride to the metal and to activate the catalyst.

After a period of service, it may be desirable to reactivate the catalyst and this may be accomplished readily by passing air or other oxygen-containing gases therethrough in order to burn carbonaceous deposits from the catalyst. A particularly suitable manner of regeneration of the catalyst comprises effecting the regeneration at a temperature of about 900° to about 950° F.,

starting with a gas containing about 2% oxygen and gradually increasing the oxygen concentration so that at the end of the regeneration period pure air is being passed over the catalyst. However, it is important that the temperature of regeneration should not exceed 1000° F. as it has been found that temperatures in excess of 1000° F. tend to impair the catalyst activity.

F. tend to impair the catalyst activity.

In carrying out reforming in accordance with this invention, temperatures in the range of 600 to 1000° F. and preferably 700 to 1000° F. may be used. The process may also be conducted at pressures from 100 to 1000 pounds per square inch and preferably at 500 to 800 pounds per square inch. Hourly space velocities (meaning the liquid volume of hydrocarbon per hour per volume of catalyst) may be in the range of 0.1 to 10, preferably in the range of 0.5 to 4. The reaction may be carried out in the presence of hydrogen in amounts from 1 to 20 mols. of hydrogen per mol. of hydrocarbon. Under these circumstances, using the instant novel catalyst it is possible to obtain from petroleum distillates, particularly gasoline fractions, yields on the order of magnitude of 88-90% or higher having motor method clear octane numbers of 71-74 or higher.

The process of the invention may be effected in any suitable equipment. An especially suitable process comprises the fixed bed process in which the catalyst is deposited in a reaction zone or zones, the hydrocarbon passing through such zone or zones and in contact with the catalyst. Another suitable apparatus in which the process may be conducted is the fluid type in which the catalyst is suspended by the gaseous hydrocarbon stream. The moving bed type process in which the catalyst and hydrocarbon are passed either concurrently or countercurrently to each other and the suspensoid type process in which the catalyst is carried as a slurry in the hydrocarbon may also be used. After reforming, the products may be fractionated to separate excess hydrogen and to recover the desired fractions of reformed product.

In one manner of operation of the process, sufficient hydrogen will be produced in the reforming reaction to maintain a hydrogen partial pressure sufficient to saturate the hydrocarbon fragments formed therein. However, hydrogen from an extraneous source is added at the beginning of the operation, and usually it is desirable to recycle hydrogen within the process after the starting operation in order to assure a sufficient hydrogen atmosphere in the reaction zone. Hydrogen serves to maintain the catalyst activity by reducing or preventing carbon deposition. Also, if desired, the petroleum distillates may be treated to remove sulfur before they are reformed.

The invention will be further illustrated in the following examples and drawings. It should be understood, however, that the examples and the drawings are given for purposes of illustration and the invention in its broader aspects is not limited thereto.

**EXAMPLE II**

10 A mixture of hydrocarbons containing by weight 46.3% of normal heptane, 44% of cyclohexane and 9.7% benzene was prepared by mixing together suitable amounts of these constituents. This mixture which is representative of  
15 the hydrocarbons contained in petroleum distillates, particularly gasoline fractions, was subjected to reforming in the presence of a silica-alumina component of varying surface areas impregnated with different percentages of platinum  
20 as indicated in Tables 1 and 2 and at the reaction temperatures indicated in these tables. The data given in Table 1 was obtained at 350 pounds per square inch pressure and that of Table 2 was obtained at 700 pounds per square inch pressure.  
25 The data in both tables was obtained using a liquid space velocity of 1. and a molar ratio of hydrogen to hydrocarbon of 4 to 1.

hydrogen to hydrocarbon of 4 to 1.

The silica-alumina component was prepared from a commercially available silica-alumina cracking catalyst. This cracking catalyst is prepared by adding sulfuric acid to commercial water glass in proportions to precipitate silica hydrogel. The silica hydrogel was washed with acidulated water to remove sodium ions, after which the hydrogel is dispersed in a sufficient amount of an aqueous solution of aluminum sulphate of suitable concentration and ammonium hydroxide is added to precipitate alumina to form a silica-alumina composite containing 13% by weight of alumina. The silica-alumina composite is then washed, dried, calcined at 600-900° F. and formed into pellets. This cracking catalyst had a surface area of 425 square meters per gram. Portions of the thus prepared silica-alumina were then treated with steam at 1050 to 1250° F. using steam pressure from 15 to 50 pounds per square inch for varying times to obtain components having the surface areas indicated in Tables 1 and 2. Solutions of chloroplatinic acid in suitable amounts and concentrations were added to the different samples of the silica-alumina composites and the thus impregnated material was dried at 220° F. and treated with a hydrogen containing gas at atmospheric pressure while the temperature was increased from room temperature to 1000° F. It was maintained at this temperature for 16 hours prior to use.

Table I

Constants: pressure: 350 p. s. i. g.; L. S. V. = 1.0; H<sub>2</sub>:HC = 4:1  
Charge: nC<sub>7</sub> (normal heptane) = 46.3; cyclohexane 44.0; benzene = 9.7 Wt. Per Cent

Table II

Constants: pressure: 700 p. s. i. g.; L. S. V.=1; H<sub>2</sub>:HC=4:1  
Charge: nC<sub>7</sub> (normal heptane)=46.3; cyclohexane 44.0; benzene=9.7 Wt. Per Cent

| Temp. ° F.<br>of<br>Reaction | Pt-0.5%<br>S. A.=425 sq. m./g. |                                       |                   | Pt-0.1%<br>S. A.=82 sq. m./g. |                                       |                   | Pt-0.05%<br>S. A.=45 sq. m./g. |                                       |                   |
|------------------------------|--------------------------------|---------------------------------------|-------------------|-------------------------------|---------------------------------------|-------------------|--------------------------------|---------------------------------------|-------------------|
|                              | Conv.<br>of nC <sub>7</sub>    | Yield<br>of C <sub>7</sub><br>Isomers | Yield of<br>Arom. | Conv.<br>of nC <sub>7</sub>   | Yield<br>of C <sub>7</sub><br>Isomers | Yield of<br>Arom. | Conv.<br>of nC <sub>7</sub>    | Yield<br>of C <sub>7</sub><br>Isomers | Yield of<br>Arom. |
| 650                          | 61.5                           | 55.3                                  | 0.0               |                               |                                       |                   |                                |                                       |                   |
| 700                          | 88.1                           | 61.0                                  | 0.1               |                               |                                       |                   |                                |                                       |                   |
| 750                          | 97.2                           | 17.8                                  | 0.6               |                               |                                       |                   |                                |                                       |                   |
| 800                          | 99.1                           | 11.2                                  | 1.0               | 70.1                          | 55.7                                  | 2.7               | 12.1                           | 12.1                                  | 0.8               |
| 850                          |                                |                                       |                   | 81.0                          | 41.7                                  | 8.9               | 28.6                           | 28.6                                  | 1.6               |
| 900                          |                                |                                       |                   | 83.9                          | 35.4                                  | 20.5              | 64.3                           | 57.9                                  | 3.0               |
| 950                          |                                |                                       |                   | 91.7                          | 12.1                                  | 26.8              | 88.7                           | 61.8                                  | 9.9               |
|                              |                                |                                       |                   |                               |                                       |                   |                                | 41.5                                  | 17.5              |
|                              |                                |                                       |                   |                               |                                       |                   |                                | 30.8                                  | 34.1              |

In the accompanying drawings,

Figure 1 is a plot of yield of C<sub>7</sub> isomers versus percent conversion of normal C<sub>7</sub> fraction for a particular surface area.

Figure 2 is a plot of conversion of normal C<sub>7</sub> fraction versus reaction temperature in degrees Fahrenheit for the catalyst of Figure 1.

Figure 3 is a plot similar to Figure 1 but with a surface area of catalyst different from that of Figure 1.

Figure 4 is a plot similar to Figure 2 but with the catalyst of Figure 3.

Figure 5 is a plot of reaction temperature in degrees Fahrenheit versus surface area of catalyst.

Figure 6 is a plot of reaction temperature in degrees Fahrenheit versus percent aromatics.

The data for the various figures were taken from Tables I and II of Example 1. Referring to the drawings, Figure 1 is a plot of yield of isomerized C<sub>7</sub> hydrocarbons versus conversion of the normal C<sub>7</sub> fraction obtained from the mixture reformed in Example I. The data for the curve of this figure is plotted for a catalyst having a surface area of 425 square meters per gram at pressures of 350 pounds per square inch (curve A) and 700 pounds per square inch (curve B). The curves of Figure 3 are similar to those of Figure 1 but are plotted for catalysts having a surface area of 45 square meters per gram, curve C representing reforming at 350 pounds per square inch and curve D, at 700 pounds per square inch. It will be noted from the curves of these figures that each catalyst of a particular surface area exhibits a maximum yield of isomerized hydrocarbon with respect to conversion of the normal C<sub>7</sub> fraction. Such maximums occur for each catalyst regardless of its surface area and pressure. For convenience and clarity in illustration catalysts having surface areas of 425 and 45 square meters per gram are shown in the curves.

In Figure 2 conversion of the normal C<sub>7</sub> fraction versus reaction temperature is plotted for the catalyst of Figure 1, curve E representing reforming at 350 pounds per square inch and curve F, at 700 pounds per square inch. Figure 4 is similar to Figure 2 but is a plot of the catalyst of Figure 3, e. g., a catalyst having a surface area of 45 square meters per gram. Curve G of Figure 4 represents the conversion versus reaction temperature curve for a catalyst having a surface area of 45 square meters per gram at both 350 pounds per square inch and 700 pounds per square inch.

The curve H of Figure 5 is a plot of reaction temperatures for the isomer yield maxima of the family of curves of which curves A and B of Fig-

ure 1 and C and D of Figure 3 are representative versus the surface area of the corresponding catalysts. The manner in which this curve was plotted is illustrated as follows: In Figure 1 the percent total conversion at which maximum isomerization of the normal C<sub>7</sub> hydrocarbons takes place, was determined from curve A by drawing the perpendicular line 1. The point at which line 1 crosses the abscissa of Figure 1 was noted. This value was then taken to Figure 2 and the horizontal line 3 of Figure 2 was drawn and extended until it intersected curve E of Figure 2. Vertical line 4 was then drawn from this point of intersection and extended to cross the abscissa of Figure 2. The point of intersection of line 4 with the abscissa of this figure was noted. This value represents the reaction temperature at which maximum yield of isomer occurs for the catalyst of curve A of Figure 1, i. e., 425 square meters per gram using 350 pounds per square inch pressure. This surface area and this temperature were then plotted in curve H of Figure 5. In a similar manner the reaction temperature for maximum isomer yield was obtained for curve B of Figure 1 and curves C and D of Figure 3 from curve F of Figure 2 and curve G of Figure 4, respectively. The other values necessary to draw curve H of Figure 5 were obtained by drawing curves similar to Figures 1 through 4 for catalysts having various surface areas. As stated earlier, for clarity and convenience of illustration, such additional curves are not shown.

It will be noted that the right hand portion of curve H of Figure 5 is relatively flat and has a very low slope while on the other hand the left hand portion of the same curve is extremely steep in slope and that the rate of change of slope of the curve increases rapidly at about a value of 65 square meters per gram at which point the inflection point of curve H occurs as is illustrated by vertical line 5.

The formation of aromatics versus reaction temperature is plotted in Figure 6. The curve J representing the formation of such aromatics at 350 pounds per square inch and the curve K for 700 pounds per square inch pressure under the reforming conditions and with the catalyst tabulated in Tables I and II. Since the mixture reformed contained 9.7% benzene all values on these curves to the right of vertical line 5 represent the production of aromatics during the conversion while those points on the curve to the left of line 5 of this figure represent destruction of aromatics substantially entirely by hydrogenation to form saturated cyclo compounds. The points at which curves J and K intersect the line 5 represent the temperatures at which the hydrogenation of aromatics and the dehydrogenation of saturated cyclo compounds is in equilib-

rium. These temperatures are determined by drawing horizontal lines 6 and 7. It will be seen, for example, that at 350 pounds per square inch this temperature is about 770° F. and for 700 pounds per square inch this temperature is about 860° F. The significance of this curve is that in order to form aromatics during reforming, it is desirable to operate above these respective temperatures for the respective pressure used. In general, the higher the reaction temperature used during conversion above these equilibrium reaction temperatures, the greater the amount of aromatics formed.

In re-examining Figure 5 in the light of the foregoing remarks with reference to Figure 6, it is seen that a catalyst having a base, the surface area of which is greater than about 65 square meters per gram is very sensitive to temperatures insofar as maximum isomer yield is concerned and that with surface areas below about 65 square meters per gram, the catalyst is substantially insensitive to temperature changes insofar as maximum isomer yield is concerned. Stated in another way, it is seen from a comparison of Figure 5 and Figure 6 that in the range of surface areas above 65 square meters per gram the temperature levels at which maximum isomerization occurs will not permit any substantial yields of aromatics, whereas in the range below 65 square meters per gram, a range of reaction temperatures exists which permits the simultaneous production of maximum yields of isomers and aromatics.

For catalysts having a high surface area the high temperatures which are desirable to obtain high yields of aromatics result in excessive, indiscriminate cracking as is illustrated by curve H of Figure 5. Such cracking largely results in demethanation or carbon deposition depending upon the amount of hydrogen present during the reforming and the pressure of such hydrogen. In general, the more hydrogen that is present and the higher the pressure that is used, the less carbon will be deposited. The advantage then of the presence of hydrogen at high pressure where cracking occurs is to reduce or substantially eliminate the deposition of carbon and to cause such cracking as occurs to be of the demethanation type. The use of high pressures, however, will require the use of even higher temperatures in order to obtain the desired amount of aromatic hydrocarbons in the reformed product. High temperatures, however, cannot be used with a catalyst having a surface area in excess of about 65 square meters per gram since with such catalysts, even in the presence of high amounts of hydrogen at high pressures, excessive cracking of the demethanation type takes place and must result in a low yield of desired liquid product due to high gas losses. Where, however, a catalyst has a low surface area, not exceeding 65 square meters per gram, high temperatures may be used to obtain high yields of aromatics and maximum yield of isomers without causing indiscriminate cracking since catalysts with such surface characteristics do not produce large amounts of gas at high temperatures.

#### EXAMPLE II

A naphtha from an Arabian crude oil having the following properties was reformed in accordance with the invention:

API gravity at 60° \_\_\_\_\_ degrees

#### ASTM distillation:

|                                      |      |          |
|--------------------------------------|------|----------|
| Overpoint                            | °F   | 167      |
| 50%                                  | °F   | 278      |
| Endpoint                             | °F   | 400      |
| 5 Clear octane number (motor method) | 37.3 | per cent |

5 Sulphur \_\_\_\_\_ per cent 0.03

A silica-alumina catalyst having a surface area of 45 square meters per gram was prepared as described in Example I. After steaming the pellets to adjust their surface area to the 45 square meters per gram, a part of them was treated as set forth in Example I to deposit thereon 0.25% of metallic platinum, the remaining portion was not so treated and contained no platinum. Both portions of catalyst were then used to reform the above identified naphtha under the following reforming conditions to give the results tabulated in Table III: 350 pounds per square inch pressure, liquid space velocity of 1, hydrogen to hydrocarbon ratio of 4 to 1 and at temperatures of 800 and 900° F.

Table III

| Temperature | Liquid Recovery, Vol. Per Cent | Clear Octane Number, Motor Method |
|-------------|--------------------------------|-----------------------------------|
| °F.         |                                |                                   |
| 800         | 98.1                           | 65.2                              |
| 900         | 90.5                           | 74.3                              |
|             | No Platinum                    |                                   |
| 900         | 98.1                           | 42.6                              |

35 The flexibility of the instant catalyst in reforming hydrocarbons by virtue of its reduced sensitivity to temperature at low surface areas of the cracking component and the importance of this discovery is therefore apparent. The present novel catalyst and process of reforming hydrocarbons with such catalyst, therefore permits the reforming of hydrocarbons to obtain high yields of a reformed product having high anti-knock characteristics.

40 The cracking component may also comprise low surface area silica-zirconia, silica-alumina-zirconia, silica magnesia, silica-alumina-magnesia, silica-thoria, silica-alumina-thoria, alumina-boria, etc., in addition to silica-alumina and such components may be impregnated with a metal containing hydrogenation catalyst such as the metals, oxides and salts of the elements of groups VI and VIII of the periodic system such as, for example, the oxides of chromium, molybdenum, tungsten and uranium, the metals, nickel, cobalt, iron and the salts thereof such as the molybdates, thiomolybdates, phosphates, tungstates, chromates and borates in addition to platinum and palladium.

45 I claim:

50 1. A process for reforming a petroleum distillate fraction boiling within the gasoline-kerosine range to increase the anti-knock value thereof which comprises subjecting said fraction to contact at reforming conditions in the presence of hydrogen with a catalyst comprising a cracking component and a metal from the group consisting of platinum and palladium, said cracking component comprising silica and alumina and having a surface area in the range of about 10 to about 65 square meters per gram of said component.

55 2. A process for reforming a gasoline fraction to increase the anti-knock value thereof which comprises subjecting said fraction to contact at

reforming conditions in the presence of hydrogen with a catalyst comprising a cracking component and a metal from the group consisting of platinum and palladium in an amount from 0.01 to 2.5% by weight of the final catalyst, said cracking component comprising silica and alumina and having a surface area in the range from about 10 to about 65 square meters per gram of said component.

3. A process for reforming a gasoline fraction to increase the anti-knock value thereof which comprises subjecting said fraction to contact at reforming conditions in the presence of hydrogen with a catalyst comprising a silica and alumina cracking component and metallic platinum in an amount from 0.01 to 2.5% by weight of the final catalyst, said cracking component having a surface area in the range of about 10 to about 65 square meters per gram of said component.

4. A process for reforming a gasoline fraction to increase the anti-knock value thereof which comprises subjecting said fraction to contact at a temperature within the range 600 to 1000° F., a pressure of from 100 to 1000 pounds per square inch, and an hourly space velocity of from 0.1 to 10, in the presence of from 1 to 20 mols. of hydrogen per mol. of hydrocarbon, with a catalyst comprising a cracking component and a metal from the group consisting of platinum and palladium in an amount from 0.01 to 2.5% by weight of the final catalyst, said cracking component comprising silica and alumina and having a surface area in the range from 10 to about 65 square meters per gram of said component.

5. A process for reforming a gasoline fraction to increase the anti-knock value thereof which comprises subjecting said fraction to contact at a temperature within the range 600 to 1000° F., a pressure of from 100 to 1000 pounds per square inch, and an hourly space velocity of from 0.1 to 10, in the presence of from 1 to 20 mols. of hydrogen per mol. of hydrocarbon, with a catalyst comprising a cracking component and metallic platinum in an amount from 0.01 to 2.5% by weight of the final catalyst, said cracking component comprising silica and alumina and having a surface area in the range from about 10 to about 65 square meters per gram of said component.

6. A catalyst comprising a component having a hydrocarbon cracking activity and a metal from the group consisting of platinum and palladium, said component comprising silica and alumina,

and having a surface area in the range of about 10 to about 65 square meters per gram of said component.

7. A catalyst comprising a component having a hydrocarbon cracking activity and a metal from the group consisting of platinum and palladium in an amount from 0.01 to 2.5% by weight of the catalyst, said component comprising silica and alumina and having a surface area in the range from about 10 to about 65 square meters per gram of said component.

8. A catalyst comprising a component having a hydrocarbon cracking activity and metallic platinum in an amount from 0.01 to 2.5% by weight of the catalyst, said component comprising silica and alumina and having a surface area in the range from about 10 to about 65 square meters per gram of said component.

9. A process for preparing a catalyst comprising heating a synthetic silica-alumina cracking component at temperatures from 1600 to 1800° F. until its surface area is reduced to about 10 to 65 square meters per gram and compositing therewith a metal from the group consisting of platinum and palladium in an amount from 0.01 to 2.5% by weight of the catalyst.

10. A process for preparing a catalyst comprising heating a synthetic silica-alumina cracking component at temperatures from 900 to 1400° F. and in the presence of steam until its surface area is reduced to about 10 to 65 square meters per gram and compositing therewith a metal from the group consisting of platinum and palladium in an amount from 0.01 to 2.5% by weight of the catalyst.

11. A process according to claim 10 in which the metal composited with the cracking component is platinum.

FRANK G. CIAPETTA.

#### REFERENCES CITED

The following references are of record in the file of this patent:

#### UNITED STATES PATENTS

| Number    | Name           | Date          |
|-----------|----------------|---------------|
| 2,375,757 | Bates          | May 15, 1945  |
| 2,399,354 | Kellett et al. | Apr. 30, 1946 |
| 2,400,465 | Marisic        | May 14, 1946  |
| 2,478,916 | Haensel et al. | Aug. 16, 1949 |
| 2,489,334 | Shabaker       | Nov. 29, 1949 |